

June 4, 1957

G. EANNARINO ET AL

2,794,943

SELENIUM RECTIFIER

Filed April 5, 1955



INVENTORS

GEORGE EANNARINO and  
ROBERT PARSONS

BY

Macen, Kalihmanen, Rithburn and Wyses.

Attorneys.

## 1

2,794,943

## SELENIUM RECTIFIER

George Eannarino and Robert Parsons, Bloomington, Ind., assignors to Sarkes Tarzian, Inc., Bloomington, Ind., a corporation of Indiana

Application April 5, 1955, Serial No. 499,271

10 Claims. (Cl. 317—241)

This invention relates to an improved selenium rectifier and to methods of preparing the same. More particularly, this invention relates to selenium rectifiers having a novel barrier layer between the selenium and the counterelectrode. More specifically, the invention pertains to selenium rectifiers wherein the barrier layer between the selenium and the counterelectrode layers is produced from a carbohydrate material and a basic organic nitrogen compound.

It is generally believed that the effective rectifying action of dry rectifiers such as selenium rectifiers, depends largely upon the formation of a barrier layer between the layer of selenium and the counterelectrode, the latter generally consisting of an alloy containing cadmium. This barrier layer is strengthened during the forming of the rectifier, which comprises applying direct or pulsating current to the rectifier in the reverse or poorly conducting direction. It has been found that the effective rectifying action of selenium rectifiers can be improved by interposing an artificial barrier layer between the selenium and the counterelectrode. In the past, this artificial barrier layer has been made of shellac, nitrocellulose, nylon, or similar film-forming organic materials.

It is the object of the present invention to provide a selenium rectifier with a novel barrier layer having improved forward and reverse characteristics. It is a further object of this invention to provide a method for producing such barrier layers in selenium rectifiers. Another object of the invention is to produce such artificial barrier layers from the combination of a carbohydrate and a basic organic nitrogen compound. These and other objects of the invention will be apparent from the following disclosure.

The invention is more readily understood by reference to the following description taken in conjunction with the accompanying single-figure drawing which shows a cross-section of a rectifier cell. The base plate 1, which may be formed of aluminum or iron, is coated with a layer of nickel 2 by electroplating or other suitable deposition method. A layer of selenium 3 is deposited on the nickel-plated base plate under heat and pressure and suitably heat-treated to form metallic selenium. On the layer of selenium, a barrier layer 4 is developed in accordance with the present disclosure, and then on top of the barrier layer 4 a counterelectrode 5 is produced.

The formation of the barrier layer is accomplished by applying to the selenium layer a thin coating of a dilute solution of a carbohydrate and an amine in a volatile aqueous solvent, allowing the solvent to evaporate leaving a residue of carbohydrate, amine and other nonvolatile organic materials on the surface of the selenium, and finally applying to the selenium layer a counterelectrode such as cadmium or a cadmium alloy. The finished rectifier cell is then electroformed by passing a relatively high current through the rectifier cell in reverse direction. The preferred method of forming the rectifier is that disclosed in the application of George

## 2

Eannarino, Serial No. 475,705, filed December 16, 1954. The forming of the cell may be conducted at low temperature or at high temperature, or both, depending upon the properties desired in the rectifier. The solution of carbohydrate and amine in volatile solvent can be applied by any suitable method, such as by spraying, or roller coating, by brushing, by applying a small amount near the center of a spinning rectifier cell, or by dipping.

The combinations of carbohydrate and organic amine which are used in forming barrier layers in accordance with the present invention are produced by forming a solution of a soluble carbohydrate in an aqueous solution of a lower alcohol and adding sufficient organic amine of the type hereinafter defined to adjust the pH to 6.5 to 7.5, and preferably 6.8 to 7.2. Higher alcohols such as furfuryl alcohol and benzyl alcohol can be added in small amounts to improve the stability of the barrier layer. Organic nitrogen compounds such as nitro-methane, nitroethane, and other lower nitroparaffins may be added in small amounts, although neither these materials nor the higher alcohols are necessary to the successful operation of the invention.

Among the carbohydrates which can be employed successfully in developing the barrier layers of this invention are sucrose, dextrose, maltose, lactose, arabinose, and similar mono- and disaccharides. These sugars can be used in pure form, or they may be used in relatively crude form as they are obtained in nature, as for example, in the form of honey or molasses. Carbohydrate derivatives such as glucuronic acid, mannitol, sorbitol, and other related materials are equally satisfactory in this invention. Polysaccharides such as starch and glycogen are operative.

The solvents for the carbohydrate solution include aqueous solutions of lower alcohols, particularly those containing 5 to 10% of water in methanol, ethanol, n-propanol, isopropanol, and the like. Mixtures of such lower alcohols may also be used. Certain other organic solvents such as acetone or methyl ethyl ketone may be employed in small quantity to assist the solution of the carbohydrate and the organic amine.

The basic organic nitrogen compounds which are suitable for use in developing the barrier layers of the present invention are those which have basic dissociation constants in the range of  $1 \times 10^{-3}$  to  $1 \times 10^{-4}$  and boiling points above 100° C. Preferred amines include the polymethylenediamines such as hexamethylenediamine, tetramethylenediamine and N,N,N',N'-tetrakis(2-hydroxypropyl)ethylenediamine. The solutions of carbohydrates and amines contain small amounts of water in the order of 1 to 10% by volume in order to aid in the interaction of the chemicals of the barrier layer with each other and with the selenium and cadmium layers. In such solutions the amount of nonvolatile materials is in the range of 0.01% to 10% by weight, and preferably in the range of 0.01% to 1%, the remainder of the solution being volatile organic solvents and water.

The counterelectrode which forms a part of the rectifier may be composed of any of the metals used in selenium rectifier counterelectrodes. In practice cadmium or cadmium alloys are preferred. The counterelectrode may be applied by evaporation under high vacuum, by spraying or by any other suitable method. Among the alloys which may be employed as counterelectrodes are cadmium-bismuth, cadmium-tin, cadmium-bismuth-lead and similar alloys melting between 90° and 300° C.

Rectifiers formed in accordance with the present invention have particularly advantageous properties. They have longer life in laboratory tests and in commercial operation than do corresponding selenium rectifiers formed by prior art methods. For example, rectifiers produced with sucrose and hexamethylenediamine have exhibited

operating lives of five to ten times as long as those of corresponding rectifiers wherein the barrier layer is produced from nylon according to the disclosure of Patent No. 2,660,698. In addition to increased life, the rectifiers are particularly stable against high humidity, high temperatures and high voltages.

The following formulations are representative of solutions within the scope of this invention which produce desirable selenium rectifiers.

*Example 1*

A solvent mixture is prepared from 780 volumes of methanol, 156 volumes of water, 31 volumes of furfuryl alcohol and 31 volumes of benzyl alcohol. To 100 milliliters of the foregoing solvent mixture are added 3 grams of crystalline sucrose. The mixture is warmed and stirred until the sucrose is completely dissolved, then cooled to room temperature. Sufficient hexamethylenediamine is added to adjust the pH to 7.0. The resulting solution is diluted with 10 volumes of 90% aqueous isopropanol.

Selenium rectifiers are prepared as follows: aluminum base plates are plated with nickel and a thin amorphous selenium coating is pressed thereon. The selenium layer is converted to metallic selenium by heat treatment. It is then sprayed with a thin coating of the above sucrose-hexamethylenediamine solution. To the dry selenium layer a thin film of bismuthcadmium alloy is applied by spraying. Rectifier cells so produced are electroformed at low temperature according to the method of the Eannarino application, Serial No. 475,705, filed December 16, 1954. The rectifiers made in this manner are uniform in performance and stable over periods of time in excess of 5,000 hours.

*Example 2*

2 grams of mannitol are dissolved in a solvent mixture containing 80 milliliters of methanol, 20 milliliters of water, 3 milliliters of furfuryl alcohol, and 3 milliliters of benzyl alcohol. Sufficient hexamethylenediamine is added to bring the pH to 7.2. The mixture is agitated and warmed nearly to its boiling point. The resulting solution is brought to room temperature and diluted 10:1 with 90% aqueous isopropyl alcohol. Rectifiers produced with this coating as in Example 1 are uniform and stable over long periods of time.

*Example 3*

2 grams of sucrose are dissolved in a solution of 20 milliliters of water in 80 milliliters of methanol. The pH of the solution is adjusted to 6.8 by the addition of N,N,N',N' - tetrakis(2-hydroxypropyl)ethylenediamine. The resulting solution is diluted with 9 volumes of 90% isopropanol. The solution thus produced forms a long-lasting barrier layer when applied to selenium.

*Example 4*

2 grams of D-glucuronic acid are dissolved in 20 milliliters of warm water. The solution is diluted with 80 milliliters of methanol and brought to pH 7.0 by titration with a 10% solution of hexamethylenediamine in methanol. The resulting solution is diluted to 1 liter with methanol and applied to selenium layers on nickel-plated aluminum base plates by spraying or rolling. The selenium layers thus treated are sprayed with cadmium-bismuth alloy and the resulting selenium rectifiers are electroformed.

Selenium layers treated as above are then coated with cadmium or cadmium alloys to a thickness of 0.001 inch to 0.01 inch. These cells are then electroformed by applying a current of relatively high current density in the range of 1 to 7 amperes per square inch in the reverse direction, either in oil solution or in air. Rectifiers produced in accordance with this invention exhibit a relatively long

life and high stability, particularly against high temperatures and humidity.

While the invention has been described in connection with specific materials and conditions, it is to be understood that this description is provided by way of illustration only, and is not a limitation of the scope of the invention.

What is claimed as new and desired to be secured by Letters Patent of the United States is:

1. A unilateral conductor comprising a base plate, a layer of selenium on said base plate, a barrier layer on said selenium layer formed by coating the selenium layer with a dilute solution containing a carbohydrate and an organic amine in an aqueous volatile solvent at a pH in the range of 6.5 to 7.5, and a counterelectrode on said barrier layer.

2. A unilateral conductor comprising a base plate, a layer of selenium on said base plate, a barrier layer on said selenium layer formed by coating the selenium layer with a dilute solution containing a carbohydrate and an organic amine having a basic dissociation constant in the range of  $1 \times 10^{-3}$  to  $1 \times 10^{-4}$  and a boiling point above 100° C. in an aqueous volatile solvent at a pH in the range of 6.5 to 7.5, and a counterelectrode on said barrier layer.

3. A rectifier comprising a base plate, a layer of selenium on said base plate, a barrier layer on said selenium layer formed by coating the selenium layer with a dilute solution containing a carbohydrate and a polymethylenediamine in an aqueous volatile organic solvent at a pH in the range of 6.5 to 7.5, and a counterelectrode on said barrier layer.

4. A rectifier comprising a base plate, a layer of selenium on said base plate, a barrier layer on said selenium layer formed by coating the selenium layer with a dilute solution containing a monosaccharide and a polymethylenediamine in a lower aqueous alcohol solvent at a pH in the range of 6.5 to 7.5, and a counterelectrode on said barrier layer.

5. A rectifier comprising a base plate, a layer of selenium on said base plate, a barrier layer on said selenium layer formed by coating the selenium layer with a dilute solution containing a disaccharide and a polymethylenediamine in a lower aqueous alcohol solvent at a pH in the range of 6.5 to 7.5, and a counterelectrode on said barrier layer.

6. A rectifier comprising an aluminum base plate, a layer of selenium on said base plate, a barrier layer on said selenium layer formed by coating the selenium layer with a dilute solution containing a disaccharide and a polymethylenediamine in a lower aqueous alcohol solvent at a pH in the range of 6.8 to 7.2, and a cadmium counterelectrode on said barrier layer.

7. A rectifier comprising an aluminum base plate, a layer of selenium on said base plate, a barrier layer on said selenium layer formed by coating the selenium layer with a dilute solution of sucrose and a polymethylenediamine in aqueous lower alcohol solvent having a pH of 6.8 to 7.2, and a cadmium alloy counterelectrode layer on said barrier layer.

8. A rectifier comprising an aluminum base plate, a layer of selenium on said base plate, a barrier layer on said selenium layer formed by coating the selenium layer with a dilute solution of sucrose and hexamethylenediamine in aqueous lower alcohol solvent having a pH of 6.8 to 7.2, and a cadmium alloy counterelectrode layer on said barrier layer.

9. A rectifier comprising an aluminum base plate, a layer of selenium on said base plate, a barrier layer on said selenium layer formed by coating the selenium layer with a dilute solution of mannitol and a polymethylenediamine in aqueous lower alcohol solvent having a pH of 6.8 to 7.2, and a cadmium alloy counterelectrode layer on said barrier layer.

10. A rectifier comprising an aluminum base plate, a

layer of selenium on said base plate, a barrier layer on said selenium layer formed by coating the selenium layer with a dilute solution of mannitol and hexamethylene-diamine in aqueous lower alcohol solvent having a pH of 6.8 to 7.2, and a cadmium alloy counterelectrode layer 5 on said barrier layer.

## References Cited in the file of this patent

## UNITED STATES PATENTS

|           |        |               |
|-----------|--------|---------------|
| 2,193,598 | Lotz   | Mar. 12, 1940 |
| 2,510,361 | Addink | June 6, 1950  |
| 2,660,698 | Black  | Nov. 24, 1953 |